# EUROPEAN PATENT SPECIFICATION

(11) **EP 1 196 515 B1**
(45) Date of publication and mention of the grant of the patent: **19.02.2003**
(21) Application number: 99936473.0
(22) Date of filing: 02.07.1999
(51) Int. Cl.: C10L 1/32

(54) **ENGINE FUELS CONSISTING OF AN EMULSION COMPRISING MINERAL AND/OR NATURAL OILS, THEIR PREPARATION AND USE IN INTERNAL COMBUSTION ENGINE**
MINERALÖL- UND/ODER NATURÖL-EMULSION ENTHALTENDE MOTORBRENNSTOFFE, DEREN HERSTELLUNG UND VERWENDUNG IN BRENNKRAFTMASCHINEN
CARBURANTS DE MOTEUR A BASE D'EMULSION RENFERMANT DES HUILES MINERALES ET/OU NATURELLES, ELABORATION, ET UTILISATION DANS DES MOTEURS A COMBUSTION INTERNE

(43) Date of publication of application: 17.04.2002
(73) Proprietor: Consorzio Interuniversitario per lo Sviluppo dei Sistemi a Grande Interfase, C.S.G.I, 50121 Firenze (IT)
(72) Inventor: BAGLIONI, Piero, I-50010 Fiesole (IT); FRATINI, Emiliano, I-59100 Prato (IT); RICCERI, Riccardo, I-50126 Firenze (IT); SARTI, Giuseppe, I-50135 Firenze (IT); CHIARAMONTI, David, I-50134 Firenze (IT)
(74) Representative: Gervasi, Gemma, Dr.
(86) International application number: EP9904607
(87) International publication number: WO01002516

(56) References cited:
- EP-A- 0 893 488
- WO-A-95/27021

## Description

### Field of the invention

The present invention refers to new fuels representing an interesting alternative to the common fossil fuels being constituted of pyrolysis liquid emulsified with natural and/or mineral oils in the presence of emulsifiers and possibly co-emulsifiers. The invention refers also to the use of the above said fuels in internal combustion engines.

### State of the art

In the last decade many studies have been performed with the aim of making available new fuels capable of replacing totally or at least in part the traditional fuels of fossil origin.

Possible substitutes of the common fossil fuels are in principle the liquids obtained by pyrolysis of biomass since they have a very low content of sulphur and therefore can be burnt without problem for the environment.

Unfortunately the oils obtained by pyrolysis contain a large amount of water (and also of acidic derivatives), are hard to ignite and present a low calorific value when compared to the fossil oils; therefore their use as such is practically impossible.

In view of the above said various works have been performed in order to realise mixture of pyrolysis liquids and the traditional fossil oils which could be industrially interesting and capable of substituting the traditional fuels.

EP-A-893 488 describes fuels in the form of pyrolysis liquid-in-diesel oil microemulsions consisting of diesel oil, pyrolysis liquid and at least an emulsifier with HLB between 4 and 18 derived from fatty acids and polyoxyethylene glycol, or fatty acids, sorbitol and polyoxyethylene or polyethoxylated alcohols with long aliphatic chains.

In spite of the good results obtained, as reported in the document, these fuels are still not completely satisfying since they require a high percentage of diesel oil in respect of pyrolysis liquid, the pyrolysis oil suitable for the preparation of the claimed microemulsions must have a limited content of water, they require the formation of microemulsions and their stability strongly depends on temperature.

It is therefore evident how it is important to make available fuels which could be used in normal internal combustion engines consisting essentially of pyrolysis liquid and not presenting the above said drawbacks.

### Detailed description of the invention

The present invention allows one to overcome the above said problems through the use of fuels consisting of emulsions of pyrolysis liquids, natural and/or mineral oils with emulsifiers and possibly co-emulsifiers capable of forming oil-in-water, water-in-oil emulsions or bicontinuous emulsions, wherein the definition emulsion does not include microemulsions.

A pyrolysis liquid (or biooil) according to the invention is the oil obtained by burning organic materials deriving from different sources and technologies according to the known techniques.

These oils normally have a content of water comprised between 20 - 45% by weight and a pH of 2,3 - 3,4.

Mineral oils are the normal oils of fossil origin like, for example, gasoline, diesel, kerosene etc.

Natural oils are the oils normally deriving as by-products from the treatment of vegetables and other oil containing natural products.

The emulsifiers play the essential role for the preparation of the fuels according to the invention.

They are chosen in the group consisting of:
- non-ionic block-copolymers (or homopolymers) surfactants having HLB from 4 to 18 possibly in combination with non ionic surfactants (co-surfactants) with HLB from 4 to 18
   and
- anionic block-copolymers (or homopolymers) surfactants having HLB 4 to 18 possibly in combination with cationic quaternary ammonium compounds.

Preferred emulsifiers of the fist group mentioned here above are:
Polyester/ether/ester block copolymers, (ABA form)
Polyether/ester/ether block copolymers, (ABA form) ,
Polyetherlester block copolymers, (AB form)
Polyether/ether block copolymers, (AB form)
Polyester/ester block copolymers, (AB form)
Polyalkylmetacrylate copolymers.

Preferred emulsifiers of the second group mentioned here above are:
Acrylic acid/ maleic acid copolymers (polycarboxylate),
Maleic acid/ olefin copolymers (polycarboxylate),
Maleic acid/ methylvinylether copolymers (polycarboxylate),
The above series crosslinked with a polyalkenyl polyether.

Quaternary ammonium compounds as defined here above are preferably monoalkyl or di-alkyl ammonium chloride surfactants wherein the alkyl chains have from C8 to C22.

The surfactants are normally added in a quantity up to 3% by weight, calculated on the total of the emulsion.

According to the invention the use of the above said emulsifier allows to emulsify oils having a water content of 20- 50%, moreover they allow the manufacture of fuels containing biooil in a range of 5 - 95% by weight calculated on the total fuel.

The fuel according to the invention present an exceptionally high stability (more than one month), their stability can even be improved by adding suitable co-surfactants.

As co-surfactants non ionic surfactants can be used according to the known techniques in order to adjust the emulsifier HLB value, and to improve the time stability of the resulting emulsion.

The co-surfactants are normally added in quantity comprised between 0,05 - 1,0% by weight calculated on the total weight of the fuel.

According to the invention the fuels can be prepared in three different kind of emulsion:
A) water-in-oil emulsion presenting a biooil/mineral or natural oil ratio of 1 - 45% (w/w)
   bicontinuous emulsion presenting a biooil/mineral or natural oil ratio of 45 - 55% (w/w)
   oil-in-water emulsion presenting a biooil/mineral or natural oil ratio of 55 - 99% w/w.

The water-in-oil emulsions are prepared by adding a surfactant of the first group indicated above to hot mineral or natural oil and thereafter adding the biooil to the resulting mixture.

Bicontinuous emulsions were formulated by adding a surfactant of the first group to the mineral or natural oil, and to the biooil and then mixing together the resulting mixtures.

Oil-in-water emulsions were formulated by adding to the biooil a surfactant (which can be chosen both in the first or the second of the above-described groups) and thereafter adding to the resulting mixture the natural or mineral oil during emulsification.

The emulsification process was carried out by using a homogeniser.

The temperature during mixing was preferably maintained between 60 - 65°C and the emulsification was continued until a homogeneous single phase was obtained. The emulsions are obtained at room temperature, too.

### Example 1

Pyrolysis oils was obtained from DynaMotive Technologies Corporation (Canada) and ENEL (Italy). In table 1 are showed the characteristics of two different employed biooils.

**Table1**

| | | |
|---|---|---|
| Moisture content (%) | 24.5 | 44.0 |
| Ash (%) | 0.03 | 0.28 |
| Density (kg/l) | 1.199 | 1.165 |
| Viscosity (mPa s) | | |
| @20°C | 55 | 10 |
| @50°C | 11 | 4 |
| Elemental | | |
| Carbon | 43.52 | 34.96 |
| Hydrogen | 6.31 | 5.94 |
| Nitrogen | 0.07 | 0.11 |
| Sulphur | 0.0 | 0.0 |
| Oxygen (diff.) | 50.07 | 58.71 |
| HHV (MJ/kg) | 16.9 | 16.5 |
| Ph | 2.4 | 3.0 |

Table 2 shows some formulations (one of each case) of prepared emulsions.

**Table 2**

| Bio-Fuel (wt%) | Diesel (wt%) | Atlox 4912 (wt%) |
|---|---|---|
| 25 | 74 | 1 |
| 49.5 | 49.5 | 1 |
| 75 | 24 | 1 |

The surfactant Atlox 4912 is a polyester/ether/ester block copolymer available from UNIQEMA.

## Claims

1. Pyrolysis oil containing fuel consisting of an emulsions of pyrolysis liquids and natural and/or mineral oils with emulsifiers and possibly co-emulsifiers capable of forming oil-in-water, bicontinuous or water-in-oil emulsions, wherein the definition emulsion does not include microemulsions.

2. Pyrolysis oil containing fuels according to Claim 1 wherein the emulsifiers are chosen in the group consisting of:
- non-ionic block-copolymers (or homopolymers) surfactants having HLB from 4 to 18 possibly in combination with non ionic surfactants with HLB from 4 to 18
and
- anionic block-copolymers (or homopolymers) surfactants having HLB 4 to 18.

3. Pyrolysis oil containing fuel according to Claim 2 wherein the content in surfactant is up to 3% by weight calculated on the total of the emulsion.

4. Pyrolysis oil containing fuels according to Claim 2 wherein the fuels is represented by a water-in-oil emulsion presenting a biooil/mineral or natural oil ratio of 1 - 45% (w/w).

5. Process for preparing a fuel according to claim 4 wherein a surfactant of the first group indicated in Claim 2 is added to mineral or natural oil and thereafter the biooil is added to the resulting mixture using a homogeniser.

6. Pyrolysis oil containing fuel according to Claim 2 wherein the fuel is represented by a bicontinuous emulsion presenting a biooil/mineral or natural oil ratio of 45 - 55%(w/w).

7. Process for preparing a fuel according to claim 6 wherein a surfactant of the first group indicated in Claim 2 is added to mineral or natural oil and to the biooil and then mixing the resulting mixtures together using an homogeniser.

8. Pyrolysis oil containing fuel according to Claim 2 wherein the fuel is represented by an oil-in-water emulsion presenting a biooil/mineral or natural oil ratio of 55 - 99% w/w.

9. Process for preparing fuel according to claim 8 wherein an emulsifier (which can be chosen both in the first or the second of the above-described groups) is added to the biooil and thereafter the natural or mineral oil is added to the resulting mixture during emulsification.

10. Pyrolysis oil containing fuel according to claim 1 containing also a co-emulsifier chosen between non ionic surfactants having HLB from 4 to 18.

11. Pyrolysis oil containing fuel according to claim 10 wherein the co-emulsifier is contained in quantity comprised between 0,05 and 0,5% w/w.

12. Pyrolysis oil containing fuel according to Claim 1 wherein the pyrolysis oil content is comprised between 55 and 99% (by weight).

13. Use of a fuel according to Claim 2 in internal combustion engines.

## Patentansprüche

1. Pyrolyseöl enthaltender Brennstoff, bestehend aus einer Emulsion von Pyrolyseflüssigkeiten und natürlichen und/oder Mineralölen mit Emulgatoren und gegebenenfalls Coemulgatoren, die Öl-in-Wasser-, bikontinuierliche oder Wasser-in-Öl-Emulsionen bilden können, wobei die Definition Emulsion keine Mikroemulsionen einschliesst.

2. Pyrolyseöl enthaltender Brennstoff gemäss Anspruch 1, wobei die Emulgatoren ausgewählt sind aus der Gruppe, bestehend aus
• nicht-ionischen Blockcopolymer (oder Homopolymer)-Tensiden mit einem HLB von 4 bis 18, gegebenenfalls in Kombination mit nicht-ionischen Tensiden mit einem HLB von 4 bis 18, und
• anionischen Blockcopolymer (oder Homopolymer)-Tensiden mit einem HLB von 4 bis 18.

3. Pyrolyseöl enthaltender Brennstoff gemäss Anspruch 2, wobei der Gehalt an Tensid bis zu 3 Gew.%, bezogen auf die Gesamtemulsion, beträgt.

4. Pyrolyseöl enthaltender Brennstoff gemäss Anspruch 2, wobei die Brennstoffe dargestellt sind durch eine Wasser-in-Öl-Emulsion mit einem Bioöl/Mineral- oder Naturöl-Anteil von 1 bis 45 % (G/G).

5. Verfahren zur Herstellung eines Brennstoffs gemäss Anspruch 4, wobei ein Tensid der ersten Gruppe gemäss Anspruch 2 zu dem Mineral- oder Naturöl zugegeben wird und anschliessend das Bioöl zu der erhaltenen Mischung unter Verwendung eines Homogenisators zugegeben wird.

6. Pyrolyseöl enthaltender Brennstoff gemäss Anspruch 2, wobei der Brennstoff dargestellt wird durch eine bikontinuierliche Emulsion eines Bioöl/Mineral- oder Naturöl-Anteil von 45 bis 55 % (G/G).

7. Verfahren zur Herstellung eines Brennstoffs gemäss Anspruch 6, wobei ein Tensid der ersten Gruppe gemäss Anspruch 2 zu dem Mineral- oder Naturöl und zum Bioöl zugegeben wird, und anschliessend Mischen der erhaltenen Mischungen unter Verwendung eines Homogenisators.

8. Pyrolyseöl enthaltender Brennstoff gemäss Anspruch 2, wobei das Öl dargestellt wird durch eine Öl-in-Wasser-Emulsion mit einem Bioöl/Mineral- oder Naturöl-Anteil von 55 bis 99 % (G/G).

9. Verfahren zur Herstellung von Brennstoff gemäss Anspruch 8, wobei ein Emulgator (der aus sowohl der ersten als auch der zweiten der oben beschriebenen Gruppen ausgewählt sein kann) zu dem Bioöl zugegeben wird und anschliessend das Natur- oder Mineralöl zu der erhaltenen Mischung während der Emulgation zugegeben wird.

10. Pyrolyseöl enthaltender Brennstoff gemäss Anspruch 1, ebenfalls enthaltend einen Coemulgator, ausgewählt aus nicht-ionischen Tensiden mit einem HLB von 4 bis 18.

11. Pyrolyseöl enthaltender Brennstoff gemäss Anspruch 10, wobei der Coemulgator in einer Menge zwischen 0,05 und 0,5 % (G/G) enthalten ist.

12. Pyrolyseöl enthaltender Brennstoff gemäss Anspruch 1, wobei der Pyrolyseölgehalt zwischen 55 und 99 Gew.% liegt.

13. Verwendung eines Brennstoffs gemäss Anspruch 2 in Verbrennungsmotoren.

## Revendications

1. Carburant contenant une huile de pyrolyse consistant en une émulsion de liquides de pyrolyse et d'huiles naturelles et/ou minérales avec des émulsifiants et éventuellement des co-émulsifiants capables de former des émulsions huile-dans-eau, bicontinues ou eau-dans-huile, dans lequel la définition du terme émulsion ne comprend pas de microémulsions.

2. Carburants contenant une huile de pyrolyse suivant la revendication 1, dans lesquels les émulsifiants sont choisis dans le groupe consistant en :
- tensioactifs à base de copolymères blocs (ou homopolymères) non ioniques ayant un HLB de 4 à 18, éventuellement en association avec des tensioactifs non ioniques ayant un HLB de 4 à 18, et
- tensioactifs à base de copolymères blocs (ou homopolymères) anioniques ayant un HLB de 4 à 18.

3. Carburant contenant une huile de pyrolyse suivant la revendication 2, dans lequel la teneur en tensioactif va jusqu'à 3% en poids par rapport au total de l'émulsion.

4. Carburants contenant une huile de pyrolyse suivant la revendication 2, dans lesquels les carburants sont représentés par une émulsion eau-dans-huile présentant un rapport biohuile/huile minérale ou naturelle de 1 à 45% en poids.

5. Procédé pour la préparation d'un carburant suivant la revendication 4, dans lequel un tensioactif du premier groupe indiqué dans la revendication 2 est ajouté à une huile minérale ou naturelle, et ensuite la biohuile est ajoutée au mélange résultant avec un homogénéiseur.

6. Carburant contenant une huile de pyrolyse suivant la revendication 2, dans lequel le carburant est représenté par une émulsion bicontinue présentant un rapport biohuile/huile minérale ou naturelle de 45 à 55% en poids.

7. Procédé pour la préparation d'un carburant suivant la revendication 6, dans lequel un tensioactif du premier groupe indiqué dans la revendication 2 est ajouté à une huile minérale ou naturelle et à la biohuile, et ensuite, les mélanges résultants sont mélangés ensemble avec un homogénéiseur.

8. Carburant contenant une huile de pyrolyse suivant la revendication 2, dans lequel le carburant est représenté par une émulsion huile-dans-eau présentant un rapport biohuile/huile minérale ou naturelle de 55 à 99% en poids.

9. Procédé pour la préparation d'un carburant suivant la revendication 8, dans lequel un émulsifiant (qui peut être choisi à la fois dans le premier ou le deuxième des groupes indiqués plus haut) est ajouté à la biohuile et ensuite, l'huile minérale ou naturelle est ajoutée au mélange résultant pendant l'émulsification.

10. Carburant contenant des huiles de pyrolyse suivant la revendication 1 contenant aussi un co-émulsifiant choisi parmi des tensioactifs non ioniques ayant un HLB de 4 à 18.

11. Carburant contenant une huile de pyrolyse suivant la revendication 10, dans lequel le co-émulsifiant est contenu en une quantité comprise entre 0,05 et 0,5% en poids.

12. Carburant contenant une huile de pyrolyse suivant la revendication 1, dans lequel la teneur en huile de pyrolyse est comprise entre 55 et 99% (en poids).

13. Utilisation d'un carburant suivant la revendication 2 dans des moteurs à combustion interne.
